

## UNITED STATES PATENT OFFICE

MARK N. FREDENBURGH, OF EAST ORANGE, NEW JERSEY, ASSIGNOR TO WESTINGHOUSE LAMP COMPANY, A CORPORATION OF PENNSYLVANIA

## LAMP MANUFACTURE

No Drawing.

Application filed August 21, 1930. Serial No. 476,951.

This invention relates to evacuated devices such as incandescent electric lamps and the like, and particularly relates to the clean-up of deleterious residual gases in such devices and comprises essentially in the provision of a specific type of clean-up material and in a method of incorporating the same within the device.

One of the objects of the present invention is to provide a heat resistant phosphorus getter admixture.

Another object of the present invention is to provide a method of incorporating the same in a coil type filament.

Another object of the present invention is to improve the exhaust of evacuated devices.

Other objects and advantages will be apparent as the invention is more fully disclosed.

In copending application by D. S. Gustin filed May 11, 1928 entitled "Process for gettering coils" is disclosed a method of applying a dry getter composition to coil type incandescent lamp filaments. Briefly described the process comprises substantially in finely comminuting the getter composition, incorporating therein the coiled filaments, and then tumbling the coils about in the finely comminuted getter material, thereby mechanically compacting the getter within the coil turns and interstices of the coiled filament. The getter composition usually employed is comprised of an admixture of phosphorus and cryolite (or sodium ferric fluoride) the phosphorus being present in the admixture in amounts varying from 1 to 30 parts.

It is customary in the manufacture of lamps and other evacuated devices, to subject the enclosing envelope to a relatively high temperature during the exhaust operation in order to effect substantial degasification of the same. With incandescent lamps this baking out temperature is dependent upon the specific glass composition and is also in part dependent upon the relative volatility and activity of the getter composition employed.

In the specific getter composition set forth by Gustin in the above identified copending application it has been found that due to the relatively fine state of subdivision of the phosphorus, that the ignition temperature of the same is relatively low. When bake out temperatures materially in excess of about 300°

C. are employed appreciable oxidation of the phosphorus is obtained, the amount thereof increasing with increased temperatures, time of exposure thereto and other factors. This progressive loss in getter material is reflected in variations in the degree of evacuation obtained by reason of the subsequent residual gas cleanup upon the flashing of the getter from the filament.

I have found that this progressive oxidation of the phosphorus during the baking out process may be substantially prevented by comprising the getter material of relatively coarse phosphorus particles and very finely comminuted cryolite (or sodium ferric fluoride), the finely comminuted cryolite serving to coat the phosphorus with a relatively adherent heat insulating coating.

I have also found that by thus comprising the getter composition of a relatively coarse and a relatively fine constituent the method of applying the same to the coil type filament must be improved in order to obtain the advantages of the dry getter method of Gustin above identified.

The specific improvement of the present invention comprises the addition of a suitable binder material to the getter composition in order to facilitate the mechanical compaction of the same within the interstices of the filament coils. The specific binder to be employed must obviously be inert with respect to the phosphorus, thermally vaporizable at relatively low temperatures without decomposition into deleterious products and readily evacuated from the device when in the vapor state. Specifically I have found that organic compounds, such as diethyl phthalate are the binder materials most suitable for the purposes of the present invention.

As a specific embodiment of the practice of the present invention I first prepare the cryolite (or sodium ferric fluoride) in a finely comminuted state by ball milling the same for a prolonged interval of time, approximately 120 hours. In this fine state of subdivision the cryolite readily passes the finest mesh, such as silk bolting cloth.

An admixture of approximately 200 grams of this material and approximately 30 grams of regular stock red phosphorus in granulated form, such as is commonly purchased upon the market, and 230 cubic centimeters of alcohol is ball milled for 30 minutes. The time interval of milling roughly controls the

particle size of the phosphorus. The milled admixture is placed on a glass tray and the alcohol evaporated at 110° C. and the dried admixture gently brushed through a 200 mesh screen and bottled. The admixture is now ready for application to the coil type filament.

The method of application of this admixture to the filament is as follows:—

- 10 Three hundred grams of metallic granulated zinc (between 20 and 40 mesh) or other suitable non-absorbent material are placed in a casserole and approximately 3 grams of diethyl phthalate is added thereto. The admixture is stirred until the zinc particles are uniformly coated with the diethyl phthalate. The binder is retained upon the surface of the zinc particles by surface tension effects. One hundred grams of the dry getter admixture is then added and the casserole and contents rotated so that the binder wetted zinc particles pick up the dry powder and cause it to adhere to the surfaces thereof by the adsorption of the diethyl phthalate.
- 25 The finished getter material will substantially comprise a quantity of round pellets made up of a core of zinc surrounded by a quantity of getter mixture. These pellets are placed in a tube or other chamber together with the coiled filaments to be gettered and the tube and contents vigorously agitated as in the Gustin process above identified. This forces the getter mixture into the core of the coil. The diethyl phthalate present acts as a binder and causes the getter mixture to pack so that future handling of the coils will not easily displace the getter.

30 During the preheating and baking out of the lamp the diethyl phthalate is vaporized completely away from the mixture. The remaining getter material comprising phosphorus in relatively coarse condition, superficially coated with inert non-inflammable 45 cryolite (or sodium ferric fluoride) withstands a higher baking temperature than the finely divided phosphorus getter composition heretofore employed.

40 This is believed due to the better heat insulation afforded the phosphorus content of the getter by the inert component surrounding the same whereby the time factor necessary to reach the kindling temperature of the phosphorus is materially increased.

55 Having broadly and specifically disclosed the present invention it is apparent that there may be many modifications made of the specific embodiment herein disclosed without departing essentially from the nature and scope of the invention as may be set forth in the accompanying claims:

What is claimed is:

1. A getter composition for evacuated devices comprising finely comminuted inert material and relatively coarse phosphorus. 70
2. A getter composition for evacuated devices comprising finely comminuted cryolite and relatively coarse phosphorus. 75
3. A getter composition for incandescent electric lamps comprising finely comminuted inert material, relative coarse phosphorus and an organic binder. 80
4. A getter composition for incandescent electric lamps comprising finely comminuted cryolite, relatively coarse phosphorus and a proportion of diethyl phthalate. 85
5. The method of gettering coil type incandescent lamp filaments comprising forming an admixture of finely comminuted inert material and relatively coarse phosphorus adding thereto a proportion of a vaporizable binder material, mechanically compacting the admixture within the interstices of said filament and evaporating the binder. 90
6. The method of gettering coil type incandescent lamp filaments comprising intimately admixing finely comminuted cryolite and relatively coarse phosphorus, adding thereto a proportion of diethyl phthalate, mechanically compacting the admixture within the interstices of said filament and evaporating the binder. 95
7. As an article of manufacture a coil type incandescent lamp filament said filament having a compact core of getter material comprising finely comminuted inert material and relatively coarse phosphorus. 100
8. As an article of manufacture, a coil type incandescent lamp filament, said filament having a compact core of getter material comprising finely comminuted cryolite, and relatively coarse phosphorus. 105
9. As an article of manufacture, a coil type incandescent lamp filament, said filament having a core of getter material mechanically compacted therein, said core comprising relatively coarse phosphorus, relatively finely comminuted cryolite and a proportion of diethyl phthalate binder. 110
10. The method of introducing a proportion of liquid binder in finely subdivided material which comprises applying said binder fluid to the surface of substantially spherical non-absorbent material to form a surface film thereon, adding the finely divided material thereto, and tumbling the admixture to obtain uniform adsorption of the binder fluid in the finely divided material. 115
- In testimony whereof, I have hereunto subscribed my name this 18th day of August 1930. 120
- MARK N. FREDENBURGH. 125